

## UNITED STATES PATENT OFFICE

FREDERICK G. MOSES, OF NEW YORK, RAYMOND W. HESS, OF BUFFALO, AND ROBERT L. PERKINS, OF EAST AURORA, NEW YORK, ASSIGNEES TO THE BARRETT COMPANY, OF NEW YORK, N. Y., A CORPORATION OF NEW JERSEY

## CONCENTRATION OF ORES BY FLOTATION

No Drawing.

Application filed May 20, 1927. Serial No. 193,055.

This invention relates to the separation of minerals and the concentration of ores by flotation processes, and is particularly directed to such separation and concentration carried out with the utilization of certain thiazole compounds or bodies as flotation agents.

According to the present invention, improved results can be obtained in the separation of minerals and the concentration of ores by carrying out the flotation operation with the addition to the ore or mineral pulp of a mercaptothiazole compound containing a monovalent organic radical as a substituent attached to one of the two adjacent carbon atoms in the thiazole nucleus.

The substituted mercaptothiazoles particularly contemplated as flotation agents or adjuvants in the process of the present invention are generally characterized by the formula



wherein R represents a hydrocarbon radical, particularly an alkyl group and especially a methyl group. It will be noted that the adjacent carbon atoms which are double-bonded to each other in the thiazole nucleus form no part of a carbocyclic ring and that R is an independent radical. The 2-mercaptop-4-methyl-thiazole is particularly important.

The mercaptothiazoles of the present invention can be prepared by methods well known in the field of organic chemistry and need no description.

In carrying out the flotation process, the flotation agent comprising a mercaptothiazole compound of the character mentioned may be incorporated with the ore or mineral pulp in any suitable manner and at any suitable time which will insure a satisfactory flotation operation. For example, it

may be introduced in the free state or as a salt into the mill in which the ore is being ground, or it may be dissolved, suspended or dispersed in any suitable solvent or dispersing agent as, for example, in one or more of the usual flotation oils or oil mixtures, or in any suitable organic solvent or medium, or in water or in an alkali or alkaline reagent, and the resulting solution, suspension or dispersion incorporated with the ore or mineral pulp. While the agents of the present invention show marked action as flotation or collecting agents in ore concentration, they generally possess insufficient frothing qualities and are therefore ordinarily used to advantage in conjunction with any suitable or well-known frothing agent, e. g., pine oil, crude turpentine, coal tar acids, etc. They may be also sometimes used to advantage in conjunction with other flotation agents. Further they may be used in the pure or purified state; or they may, in general, be also employed in the crude state.

The process of the present invention can be carried out in any suitable apparatus, for example, those of the pneumatic type such as the Callow cell, or those where the air is incorporated with the mixture by agitation such as the Janney apparatus, or the like.

It is of advantage in some cases, as with certain copper ores, to subject the ore pulp to the action of an amount of alkali sufficient to give it an alkaline reaction before subjecting it to flotation with the aid of the flotation agents of the present invention. The alkali may be caustic alkali such as caustic soda, or an alkaline salt such as soda ash, or it may be calcium oxide or hydrate.

In the differential separation of various minerals, such as zinc blende from associated minerals, the presence of an alkali metal cyanide, or of copper sulfate or other salts, is sometimes advantageous.

The amount of flotation agent required

to be used in the flotation process will vary, it depending partly on the character and composition of the ore, partly on the particular mercaptothiazole derivative employed, and partly on other factors. In many cases, one-sixth to one-half pound of the flotation agent per ton of dry ore will be sufficient, while in other cases larger or smaller amounts than this may be required.

10 The invention will be further illustrated by the following specific example, but it will be understood that the invention is not limited thereto. The parts are by weight.

Example: 500 parts of a copper sulfide ore (of the Miami Copper Company) assaying 1.27 percent copper was ground in a ball mill with 300 parts water and 0.75 parts hydrated lime (equivalent to 3 pounds per ton of ore) until practically all of it was 20 sufficiently fine to pass a 40-mesh screen. The ground pulp was diluted with sufficient water to give a pulp containing about 16 percent solids and subjected to flotation in a Janney mechanical apparatus with the 25 addition of 0.0625 parts of 2-mercaptop-4-methylthiazole (equivalent to one-fourth pound per ton of ore) previously dissolved in an equivalent amount of normal caustic soda solution. The mixture was agitated 30 for 30 minutes during which time about 0.06 parts of pine oil was introduced. 21.2 parts of a concentrate assaying 22.9 percent copper was obtained which is a recovery in the concentrate of 77.6 percent of copper. The 35 tailings assayed 0.31 percent copper. It will be noted that the equivalent of about 23.4 tons of ore was required to give one ton of concentrate.

It will thus be noted that the present invention contemplates the utilization of substituted mercaptothiazole bodies as flotation agents; that said flotation agents may be incorporated in or with the ore in any suitable manner; that they may be used in conjunction with other flotation agents or with frothing agents, or with both; and that they may be used in the free state or as salts, or in solution, suspension or dispersion in any suitable solvent or medium.

50 The present invention is of more or less general application to the treatment of different kinds of mineral substances, both natural and artificial, by flotation.

It will be further understood that the invention is not limited to the use of the particular agents or ingredients mentioned in the example and that other agents, particularly other flotation agents of the class specified, can be similarly used.

60 We claim:

1. In effecting the concentration of minerals by flotation, the process which comprises incorporating with the mineral pulp a mercaptothiazole compound containing a monovalent organic radical as a substituent

attached to the thiazole nucleus, and subjecting the resulting mixture to a froth flotation operation.

2. In effecting the concentration of minerals by flotation, the process which comprises incorporating with the mineral pulp 70 a mercaptothiazole compound containing a monovalent hydrocarbon radical as a substituent attached to the thiazole nucleus, and subjecting the resulting mixture to a froth 75 flotation operation.

3. In effecting the concentration of minerals by flotation, the process which comprises incorporating with the mineral pulp 80 a mercaptothiazole compound having in the free state the probable formula



wherein R denotes a hydrocarbon radical, 85 and subjecting the resulting mixture to a froth flotation operation.

4. In effecting the concentration of minerals by flotation, the process which comprises incorporating with the mineral pulp 90 a mercaptothiazole compound having in the free state the probable formula



wherein R denotes an alkyl group, and subjecting the resulting mixture to a froth 95 flotation operation.

5. In effecting the concentration of minerals by flotation, the process which comprises incorporating with the mineral pulp 100 a mercaptothiazole compound having in the free state the probable formula



105

and subjecting the resulting mixture to a froth flotation operation.

6. In effecting the concentration of minerals by flotation, the process which comprises subjecting a copper sulfide ore in the form of a pulp to a froth flotation operation in the presence of a mercaptothiazole having in the free state the probable formula:



110

wherein R denotes a hydrocarbon radical.

7. In effecting the concentration of minerals by flotation, the process which comprises subjecting a copper sulfide ore in the form of a pulp to a froth flotation operation 120 in the presence of a mercaptothiazole having in the free state the probable formula:



125

wherein R denotes an alkyl group.

8. In effecting the concentration of minerals by flotation, the process which com- 130

prises subjecting a copper sulfide ore in the form of a pulp to a froth flotation operation in the presence of a mercaptothiazole having in the free state the following probable formula:



5 In testimony whereof we affix our signatures.

10 FREDERICK G. MOSES.  
RAYMOND W. HESS.  
ROBERT L. PERKINS.

prises subjecting a copper sulfide ore in the form of a pulp to a froth flotation operation in the presence of a mercaptothiazole having in the free state the following probable formula:



In testimony whereof we affix our signatures.

10 FREDERICK G. MOSES.  
RAYMOND W. HESS.  
ROBERT L. PERKINS.

15

CERTIFICATE OF CORRECTION.

Patent No. 1,806,362.

Granted May 19, 1931, to

FREDERICK G. MOSES ET AL.

It is hereby certified that error appears in the printed specification of the above numbered patent requiring correction as follows: Page 1, in the last line of the formula between lines 21 and 25, for "N" linked to the 5 C atom read H; and that the said Letters Patent should be read with this correction therein that the same may conform to the record of the case in the Patent Office.

Signed and sealed this 7th day of July, A. D. 1931.

M. J. Moore,  
Acting Commissioner of Patents.

(Seal)

45

50

55

60

65

**CERTIFICATE OF CORRECTION.**

**Patent No. 1,806,362.**

**Granted May 19, 1931, to**

**FREDERICK G. MOSES ET AL.**

**It is hereby certified that error appears in the printed specification of the above numbered patent requiring correction as follows: Page 1, in the last line of the formula between lines 21 and 25, for "N" linked to the 5 C atom read H; and that the said Letters Patent should be read with this correction therein that the same may conform to the record of the case in the Patent Office.**

**Signed and sealed this 7th day of July, A. D. 1931.**

**(Seal)**

**M. J. Moore,  
Acting Commissioner of Patents.**